

July 13, 1937.

W. H. MOSS

2,086,729

OPTICAL SCREEN AND MATERIAL USED IN THE MANUFACTURE THEREOF

Filed Aug. 10, 1934

FIG. 1



FIG. 2



FIG. 3



Inventor:  
William H. Moss  
by  
J. Seltzer and B. F. Fennom  
Attorneys

## UNITED STATES PATENT OFFICE

2,086,729

OPTICAL SCREEN AND MATERIAL USED IN  
THE MANUFACTURE THEREOFWilliam Henry Moss, London, England, assignor  
to Celanese Corporation of America, a corpora-  
tion of DelawareApplication August 10, 1934, Serial No. 739,239  
In Great Britain September 1, 1933

3 Claims. (Cl. 88—24)

This invention relates to optical screens, and in particular to translucent projection screens such as are used, for example, in cinematography and allied arts.

Translucent projection screens such as are used in cinematography, for example where it is required to provide a back-ground for a scene being photographed, have hitherto been constructed of glass. The screens in question are often required to be of large dimensions and the manufacture of such screens from glass, particularly since the surface is required to be substantially plane, is attended by considerable expense. It is the primary object of the present invention to avoid this and other disadvantages of the use of glass, among which may be mentioned liability to breakage and undesirable weight, by substituting for glass a more suitable material and modifying the construction of the screen accordingly. In the case of rigid or semi-rigid unbreakable glass substitutes, difficulty is encountered in ensuring that the surface shall be plane, particularly in view of the tendency of many of such materials to warp. The present invention contemplates a material which shall be sufficiently strong and flexible to be stretched so as to provide a plane surface. I have found that very satisfactory screens can be made from sheets of flexible translucent material comprising a textile fabric, having its interstices filled with an artificial film-forming substance.

The present invention therefore comprises optical screens, the sheet material of which comprises a textile fabric having its interstices filled with an artificial film-forming material. The fabric forming the basis of the sheet material of the screen is preferably a plain woven one, but special means may be adopted in weaving to reinforce the fabric so as to enable it to withstand the tension necessary to stretch it so as to provide a plane surface. With this object in view the fabric may be reinforced by a strong selvedge and by extra strong wefts at the ends. Stretching of the fabric may be facilitated by turning over each edge in the form of a hem into which can be inserted a suitable member, e. g. a metal rod or lath, to which the tension can be conveniently applied. The hems, instead of being continuous so that the laths have to be gripped at their ends, may have openings in them at intervals through which the laths may be gripped, e. g. by cords or wires attached to tensioning means. When the material of the fabric is thermoplastic, heat and pressure may be applied to cause the yarns of the hem to co-

alesce so that the laths are vertically embedded in the fabric. Instead of laths or rods, strong cords or wires, having loops or eyes at intervals along their lengths may be worked into the fabric along each side to facilitate tensioning. Again the fabric, if a thermoplastic one, may be consolidated under heat and pressure at the edges, so as to embed the cords in the material.

The fabric forming the basis of the sheet material preferably has a basis of cellulose acetate. Other thermoplastic filament-forming substances may, however, be employed, among which mention may be made of other organic esters of cellulose, for example cellulose formate, propionate or butyrate, ethers of cellulose, for example ethyl, methyl, benzyl cellulose, ether-esters of cellulose, for example oxyethyl cellulose acetate, esters of cellulose containing inorganic radicles, for example nitrocellulose and cellulose nitroacetate, and thermoplastic derivatives having a noncellulosic base, for example polymerized vinyl acetate and other polymerized vinyl compounds. The yarns of cellulose acetate or other thermoplastic material used in the manufacture of the fabric may be produced by a wet or dry spinning method. Since high tensile strength is of advantage for the materials used in the present invention, it is preferable to employ in the manufacture of the yarns base materials which are particularly adapted to produce yarns of high strength, and/or to subject the yarns during or after their production to processes which enhance their tensile strength. Thus base materials of relatively high viscosity may be employed with advantage. For example, in the case of cellulose acetate, the yarns from which the fabric is made may have a viscosity of the order of 30, and may with advantage have a considerably higher viscosity, for example 50 or even 100 or more, these viscosities being arrived at by comparison of the viscosity of a 6% solution of the cellulose acetate in acetone with glycerine at the same temperature. In spinning the yarns, special methods may be adopted with a view to obtaining a high tensile strength. The spinning may, for example, be carried out by one of the processes of U. S. applications S. Nos. 402,735 filed 26th October, 1929, 418,414 filed 3rd January, 1930, 437,423 filed 20th March, 1930, 469,622 filed 21st July, 1930, and 601,043 filed 24th March, 1932, in which a considerable draw-down is applied during spinning. Again, the yarns may, continuously with or after their production, for example by a dry spinning process, be stretched in the presence of stretch-assisting

agents to a relatively great extent, for example to 200% or even 500% or more of their original length. Further, cellulose ester materials may be partially saponified and this process may be effected so as to enhance the tensile strength of the materials. The yarns used in the manufacture of the fabric may have a tensile strength of 2.5, 3 or even 4 or more grams per denier. However, yarns of much lower tensile strength, e. g. 1.5-2 grams per denier or even less may be used.

Although it is preferable to employ as the material for the base fabric a thermoplastic substance, the fabric may be made from non-thermoplastic materials, for example from artificial materials of the regenerated cellulosic type, for example viscose artificial silk, cuprammonium artificial silk, or the materials obtained by the complete saponification of organic esters of cellulose, which may have a very great tensile strength. The yarns used in such fabrics may be produced by any convenient process, but again due regard should be had to the desirability of obtaining materials of relatively high tensile strength. In the case of regenerated cellulosic materials of the viscose or cuprammonium type, it is of advantage in view of this object to treat the formed materials with, or even to form them in the presence of, concentrated mineral acids, for example sulphuric or hydrochloric acid, preferably while they are under tension. Such processes may be carried out so as not only to increase the strength of the materials but also to render them translucent or even transparent if they are not already so. This is a point of importance since whatever the nature of the fabric employed it should preferably be naturally translucent or transparent, or capable of being rendered so at some stage in the manufacture of the sheet material, for example by treatment with the film-forming substance employed to fill up the interstices in the fabric. Cellulose acetate and similar derivatives of cellulose may be prepared in a form sufficiently translucent for the present purpose without further treatment. Moreover, treatment of such materials with, for example, polymerized vinyl acetate, which may form the basis of the material used in filling the interstices in the fabric, may render them even transparent. Materials having a cellulosic base, however, may require some special treatment such as that indicated above. The yarn may, before or after it is made into fabric, be treated with a substance adapted to decrease its opacity, e. g. an oil, fat or wax, or a natural or synthetic resin. Such substances may even in some cases be introduced into the dope from which the yarn is spun. The last method is however of limited application since in many cases such substances are incompatible either with the filament-forming material itself or with other constituents of the spinning solution, and tend to become dispersed throughout the material and to decrease its lustre without achieving the result desired. A more generally useful method in the case of wet spun products is to introduce such substances into the coagulating bath or in wet or dry spinning processes to apply them, for example in a bath or by means of padding rolls or a wick, to the spun materials continuously with their production. On the other hand, particularly when the film-forming composition is adapted to decrease the opacity of the fabric, it may even be of advantage to subject this to processes adapted to increase the opacity or to apply

such processes in the manufacture of the yarns. Thus, for example, substances incompatible with the base of the materials may be distributed throughout the filaments, for example by introduction into the spinning solution, or methods such as those outlined below may be used. Whatever method is employed, however, care should be taken that the strength of the filaments is not unduly affected.

The fabric may be made from a fibre of natural origin, for example a cotton, linen or other vegetable fibre. In this case also the material may with advantage be subjected to the action of strong mineral acids and to other processes directed to decreasing the opacity of the material. Further, materials of vegetable origin may, if desired, be mercerized, preferably under tension, or subjected to other superficial treatments, e. g. immunization.

The film-forming substances employed to fill up the interstices of the fabric are preferably thermoplastic substances such, for example, as those listed above in connection with the fabric. Excellent results have been obtained, particularly where the fabric was composed of cellulose acetate by the use of polymerized vinyl acetate as the film-forming substance. The substance employed may be of the same chemical nature as that from which the fabric is made, but it is of advantage, with a view to its application to the fabric without damage thereto, that it should have different solubility characteristics. For example a fabric made of acetone-soluble cellulose acetate may readily be coated with a composition containing a cellulose acetate of different solubility characteristics dissolved, for instance, in ethyl acetate, without danger of the solvent attacking the fabric. Again, a cellulose acetate of high acetyl value, soluble in ethylene methylene ether may be used for the film-forming composition when the fabric comprises a cellulose acetate of lower acetyl value insoluble in ethylene methylene ether. It is of considerable advantage for the film-forming substance to be soluble in volatile solvents, so that it can be applied in solution in such solvents, for example by spraying, by extrusion on to the moving fabric in an evaporative atmosphere, by spreading, or by a bath treatment the solvent being removed by evaporation leaving a coherent coating of film-forming material between the interstices of the fabric. A film-forming substance which is soluble in volatile solvents may even be applied to a fabric comprising a substance of the same solubility characteristics without damage, by spraying methods such that the solvent evaporates very rapidly, so that the composition impinging on the materials contains no more solvent than is required to produce a coherent coating. The liquid composition containing the film-forming substance may contain plasticizers therefor which should preferably be compatible with the material of which the fabric is composed. A large number of plasticizers are available for use with polymerized vinyl esters or the like and/or cellulose acetate and like derivatives of cellulose. Among these mention may be made of sulphonamides, for example toluene ethyl sulphonamide and the isomeric xylene monomethyl sulphonamides, organic tartrates, for example dibutyl or dibenzyl tartrate, organic phthalates, for example diethyl or dibutyl phthalate, esters of polyhydric alcohols, for example triacetin, the phosphates of phenolic and substituted phenolic bodies, for example tri-resorcinol phosphate and the phosphates of halo-

generated phenols or naphthols, condensation products of phenols or naphthols or their homologues or substitution products, for example chlor-phenols with ketones including aliphatic 5 and cyclic ketones, for example acetone cyclohexanone, methyl cyclohexanone, cyclopentanone, cycloheptanone and other ketones of the cyclo paraffin series. Corresponding with diphenyol propane other diphenyol or substituted 10 diphenyol substitution products of methane hydro-carbons or of substituted methane hydrocarbons may be used, the substitution being either by alkyl or aryl groups, as for example in di-para-oxy-phenyl-diphenyl-methane (obtainable 15 by condensation of benzophenone dichloride with phenol). Again the solid intermediate condensation products of furfural or benzaldehydes or other aliphatic or cyclic aldehydes with acetone or other ketones including cyclic ketones 20 may be used, the term intermediate product being used to denote the more or less crystalline chemical compounds obtainable before the condensation is carried out sufficiently far to produce a wholly resinous product. Other compounds 25 which may be employed are alkyl derivatives of phenol, for example tertiary butyl phenol. The amount of plasticizer employed will depend upon the natural flexibility of the substance forming the base of the film-forming composition. Pro- 30 portions of 20, 30 and 50% have been used with success where the base of the film-forming composition is a polymerized vinyl acetate and even higher proportions may be used provided the resulting coating is not thereby rendered sticky. 35 Further, the compositions may contain synthetic resins, for example the resin obtainable by condensation of formaldehyde with diphenyol propane or with the crude condensation product of phenol and acetone. Very useful compositions 40 are those, for example, prepared with the aid of polymerized vinyl acetate, an equal or somewhat smaller amount down to half the quantity of diphenyol propane formaldehyde resin and a quantity of tricresyl phosphate about equal to 45 the quantity of diphenyol propane formaldehyde resin. Similarly the resins formed by condensation of diphenyol propane with furfural or with aldehydes may be used, or the resinous condensation products of formaldehyde, furfural or other aldehydes with other condensation products of ketones and phenols, including the condensation products of phenols with the ketones of the cyclo paraffin series, such as cyclo hexanone, cyclo pentanone and the like. Again the 50 resinous products obtainable from phenolic bodies and acetone or other aliphatic ketones or the cyclo paraffin ketones such as cyclo hexanone may be used, and in addition the synthetic resins obtainable from furfural or other aldehydes and acetone or other ketones. The compositions may, moreover, contain sulphonamide 55 aldehyde resins, urea formaldehyde resins or the resins obtained by condensation of glycols, glycerine and other polyhydric alcohols or derivatives thereof with phthalic acid, phthalic anhydride or other polybasic acids or anhydrides. The compositions may contain substances adapted to decrease the inflammability of the material, and the presence of such substance is of particular 60 value where the film-forming base or the material of which the fabric is made is a highly inflammable substance such as nitro-cellulose. The substance employed to decrease the inflammability of the material may comprise a halogenated 65 organic compound or a compound capable, on

the application of heat, of evolving a non-inflammable gas, for example an ammonium salt. The non-inflammators used may, as in the case, for example, of trichlor- and tribromacetanilides, themselves be plasticizing or softening agents for 5 the film-forming substance.

Other film-forming substances which may be used include polymerized acrylic esters and similar polymerized esters of unsaturated acids and alkyde resins, preferably modified by heating with 10 higher fatty acids or glycerides thereof.

Although it is preferable to employ for the film-forming substance to be applied to the fabric a thermoplastic substance which is soluble in volatile organic solvents, non-thermoplastic substances may be used. I may, for example, deposit cellulose upon the fabric from solutions containing cellulose or unstable cellulose derivatives, for example from viscose or cuprammonium solutions of cellulose. Such materials are preferably 20 employed when the fabric forming the base of the sheet material itself consists of or contains cellulose or regenerated cellulose threads. The viscose or cuprammonium cellulose may conveniently be applied to the fabric by extruding 25 the solution on to the fabric while it is passing through a bath containing a suitable coagulating agent which must not, of course, be of such a nature as to affect the fabric deleteriously.

Dyes may be applied to the sheet material of 30 the screens either for the purpose of obtaining coloured screens which are desired for certain purposes or for obtaining special effects such as a screen of increasing opacity towards the centre as referred to hereinafter. For coloured screens 35 the dyestuff may be applied uniformly over the sheet material or locally, depending upon the effect desired, and of course multi-colour effects may be produced in any desired design. The dyestuffs may be included in the film-forming 40 composition applied directly to the fabric or may be included in a special surfacing composition.

The sheet material should preferably have a matt finish on one or both sides. This may be applied in various ways, depending upon the nature of the material. A convenient method which is of general application is to apply to the coated fabric a further coating composition containing cellulose acetate or other, preferably 45 thermoplastic, film-forming substance, preferably in solution in a volatile solvent or solvent mixture, and a finely divided colourless or white insoluble material. I have obtained the best results in connection with fabrics the interstices of which have been filled with a composition containing a polymerized vinyl acetate by applying as a finish a composition containing cellulose acetate dissolved in a volatile solvent in which is suspended finely divided silica. Among other 50 finely divided materials which may be used are barium hydroxide, zinc oxide, titanium dioxide, talc, and other white or colourless heavy metal oxides, hydroxides and silicates. Insoluble organic compounds of high melting point, such as 55 are referred to in U. S. application S. No. 473,781 filed 7th August, 1930, can also be used. Instead of applying the finely divided materials in the form of an additional coating upon the already 60 coated fabric, they may be incorporated in the film-forming composition with which the interstices of the fabric are filled. In this event, however, unless the thickness of the sheet is considerably greater than that of the fabric, there is 65 some possibility of an uneven effect being produced in the sheet material owing to those parts 70 75

of it corresponding to the interstices of the fabric containing a greater amount of finely divided substance than the parts corresponding to the warp and weft. This effect may be to some extent eliminated by subjecting the fabric to pressure, preferably at elevated temperature, e. g. by passing it between heated rolls or through a platen press, so as to flatten the warp and weft yarns and, if the treatment is applied after the application of the film-forming composition, in addition distribute the coating composition containing the finely divided substance more evenly over the whole fabric. Instead of coating the material with a composition containing a finely divided material the matt effect may be produced in the case of material coated with cellulose acetate or like thermoplastic or film-forming substances simply by subjecting of the sheet to pressure, preferably at elevated temperatures. It may, for example, be passed between rolls which may be heated and/or suitably engraved. Again, where the coating comprises cellulose acetate or like substances, a matt effect may be produced by subjecting the material to the action of moist steam. A method of wider application, and capable in fact of use whatever the nature of the coating composition, is to subject the surface of the material to abrasion. A further method applicable when the material is soluble in organic solvents is to subject it to treatment with a liquid composition containing a solvent in such concentration as to pit the surface of the material. Again, the material may be coated with a film-forming substance in form having a discontinuous internal structure, e. g. cellulose acetate deposited from an aqueous bath in the absence of swelling agents, salts or other substances which tend to assist the formation of a continuous gel structure.

For certain purposes it is desirable to have the centre portion of the screen more opaque than the peripheral portions. This effect may be obtained by applying to the centre portion a heavier coating of the matt surfacing material. A similar effect may be obtained by applying to the centre portion a clear coat containing a suitable dye.

The stretching of the sheet material to obtain a plane surface may be effected during its manufacture. The fabric may, for example, be clamped into a suitable frame while held under tension in two directions at right angles. The film-forming composition and/or any finishing composition desired may then be applied to the material, preferably by spraying, while it is still stretched in the frame. Alternatively, the material may be clamped in a frame under substantially no tension and the requisite tension may be obtained by the careful application of a shrinking agent, for example, when the fabric is of cellulose acetate or the like, one of the substances referred to in U. S. application S. No. 611,240 filed 13th May, 1932. On the other hand, the stretching of the sheet material may take place as the last stage in the manufacture. Any convenient stretching means may be employed. The material may, for example, be held between jaws, the distance apart of which can be varied by means of screws, or attached to rollers by rotation of which tension can be applied, so as to stretch the fabric until it presents a plane surface. Or, as indicated above, the edges of the fabric may be provided with rods or laths for the application of the tension. Such rigid members may be held apart, for example, by

means of cords or struts, particularly struts which are hinged so as to produce a toggle effect. When the fabric is provided along its edges with eyelets or loops, they may be attached to suitable tension devices, for example springs, rollers, 5 rotatable pegs or levers, by means, for instance, of cords, wires or the like.

The following is an example of the manufacture of a fabric suitable for use in the production of the screens of the invention. 10

#### Example

A cellulose acetate woven fabric having a weight of about 1.6 ounces per square yard is stretched 15 and fastened on to a wooden frame. It is then coated with a vinyl acetate dope on both sides by spraying so as to give a weight of about 4 ounces per square yard of dry film. This has the effect of making the cellulose acetate almost transparent. 20 The dope used in coating has the following composition:—

|                                   |        |     |    |
|-----------------------------------|--------|-----|----|
| Vinyl acetate of medium viscosity | ounces | 4.5 | 25 |
| Amyl acetate                      | ccs    | 540 |    |
| Butyl alcohol                     | ccs    | 56  |    |
| Toluene                           | ccs    | 336 |    |

The fabric is dried, after which a dope of the 30 following composition is sprayed on to one or both sides:

|                       |       |      |    |
|-----------------------|-------|------|----|
| Cellulose acetate     | grams | 120  |    |
| Dibutyl tartrate      | grams | 30   | 35 |
| Acetone               | ccs   | 150  |    |
| Benzene               | ccs   | 84   |    |
| Alcohol               | ccs   | 66   |    |
| Ethyl lactate         | ccs   | 37.5 |    |
| Finely divided silica | grams | 47   | 40 |

The effect of this coating is to give the material a semi-opaque translucent surface.

The accompanying drawing illustrates diagrammatically tensioned optical projection screens in 45 accordance with the present invention.

In Fig. 1 the fabric 4 coated as above described and provided with reinforced edges 5 and eyelets 6 in the reinforcement is held by means of the eyelets 6 and the springs 7 to the frame 8. In Fig. 2 the fabric 4 has cords or wires 9 stitched or otherwise attached thereto. In the case of a thermoplastic fabric the cord or wire may, as previously described, be embedded in the material by means of heat and pressure. The cords or 55 wires 9 are continued out of the fabric as cords or wires 10 for tensioning purposes. The fabric is of course coated as previously described. In Fig. 3 the fabric 4, coated as previously described, is provided with hems 11 through which are passed stiff laths or rods 12 for holding the fabric taut. As previously described the hems may have openings in them to enable the rods or laths to be gripped at intervals by cords or wires.

What I claim and desire to secure by Letters 65 Patent is:—

1. Translucent optical projection screens comprising a sheet of an organic derivative of cellulose textile fabric having its interstices filled with a film-forming material comprising a polymeric vinyl compound and having at least one matt surface, and means for maintaining the said sheet under tension.

2. Translucent optical projection screens comprising a sheet of a cellulose acetate textile fabric 71

having its interstices filled with polymerized vinyl acetate and having at least one matt surface, and means for maintaining the said sheet under tension.

5. Translucent optical projection screens comprising a sheet of a cellulose acetate textile fabric having its interstices filled with a polymeric

vinyl compound, at least one surface of the said sheet being coated with a cellulose derivative composition containing finely divided silica, and means for maintaining the said sheet under tension.

WILLIAM HENRY MOSS.